

# United States Patent Office

3,290,183

Patented Dec. 6, 1966

1

3,290,183

## METHOD OF PRODUCING ANTICORROSION HIGH TENSILE STRENGTH RAIL

Tadashi Ohtake, Tobata, Fukuoka; Koichi Aoki, Yawata, Fukuoka, and Isao Kimura, Tobata, Fukuoka, Japan, assignors to Yawata Iron & Steel Co., Ltd., Tokyo, Japan, a corporation of Japan

Claims priority, application Japan, Aug. 29, 1961,

36/31,225

No Drawing. Filed Aug. 21, 1962, Ser. No. 218,429

3 Claims. (Cl. 148—12)

The invention relates to method for producing corrosion-resistant high tensile strength rails.

Rails actually used in every country today are largely classified with respect to their compositions as high carbon steel rails and low carbon medium manganese steel rails. In Japan, most of the rails are carbon steel rails which are intermediate between the above mentioned two kinds. In some parts of Europe and America, rails containing very small amounts of Cr and V or Si-Mn series have been experimentally manufactured in order to obtain fatigue-resistance or high tensile strength. However, these rails contain only small amounts of alloys and are not intended to have corrosion-resistance. In carbon steel rails used today, the amount of breaks due to both corrosion and fatigue and due to corrosion and electrolytic corrosion are very high. On the other hand, the fatigue limit of current carbon steel rails is 30 to 35 kg./mm.<sup>2</sup>. But, in old rails which have been used to some extent, the fatigue limit decreases due to their exposure to corroding environments. Current rails are not yet satisfactory with respect to corrosion and fatigue-resistance.

An object of the present invention is to completely eliminate the defects of conventional rails with respect to corrosion and fatigue-resistance and to provide rails having high corrosion and fatigue-resistance.

Another object of the present invention is to give toughness and anticorrosion to rolled rails and to provide rails in which the production of flakes is prevented.

The rail according to the present invention is composed of about 0.05 to 0.25% C, about 2.0 to 6.0% Cr, less than about 1.0% Mo, less than about 1.5 Mn, less than about 1.0% Si and the remainder being Fe and unavoidable impurities and may, according to circumstances, contain less than about 1.0% Ni, less than about 0.5% V, less than about 1.0% Cu, less than about 0.01% B, less than about 0.5% Ti and/or less than about 0.5% Nb.

In the rail of the present invention, high toughness and corrosion-resistance are achieved by properly controlling the cooling rate of the rail after rolling it, or by tempering the rail after cooling to room temperature.

The rail according to the present invention can contain carbon in a range of about 0.25 to 0.05% in view of its self-hardenability and the precipitation of carbide at high

2

temperatures. The chromium content in the rail of the present invention is about 2.0 to 6.0% to give corrosion-resistance and strength. When the chromium content is less than about 2%, there is very little corrosion-resistance. When it is more than about 6%, corrosion-resistance does not increase sufficiently to make the rail economical. Molybdenum greatly improves both strength and toughness. In the present invention, the molybdenum content is less than about 1% or preferably about 0.1 to 0.4%. Less than about 1.0% of each of nickel, vanadium, boron, copper, titanium and niobium may be added to increase the strength and toughness or corrosion-resistance but they are not necessary ingredients.

In producing the rail of the present invention, a steel ingot having the above composition is bloomed, is then slowly cooled, is reheated and is then rolled into a rail and the rail is then cooled at a properly controlled cooling rate, or the rail cooled to room temperature is then tempered.

When the rail of the present invention is rolled and is then cooled in air, the hardening rate is so great that the rail becomes very brittle. Further, because of the rail's strong tendency to flake the finish-rolled rail is slowly cooled to obtain toughness and to prevent the formation of flakes. By such heat-treatment, the formation of flakes is prevented, toughness is attained and, at the same time, corrosion and fatigue-resistance are increased. For such heat-treatment after rolling the rail, it is preferable to put the rail into a heat keeping furnace or a soaking pit when the temperature of the rail has reached about 750 to 500° C. during the air-cooling. The rail is slowly cooled therein for more than about 7 hours to about 200 to 150° C. The rail can thereafter be air cooled to room temperature after the finish roll then tempered at about 400 to 800° C. and again air-cooled. By this procedure, rails high in corrosion-resistance, toughness and fatigue-resistance are obtained.

Blooming or rolling of rails can be replaced by other processes such as, for example, pressing, extrusion or forging.

Table 1 shows the chemical compositions of a corrosion-resistant high tensile strength rail according to the present invention and of a current carbon steel rail. Table 2 shows the results of tests conducted with the said rails.

Table 1

|                               | C    | Si   | Mn   | P     | S     | Cr   | Mo   |
|-------------------------------|------|------|------|-------|-------|------|------|
| Rail of the present invention | 0.09 | 0.21 | 0.67 | 0.013 | 0.020 | 4.90 | 0.42 |
| Current carbon steel rail     | 0.65 | 0.13 | 0.81 | 0.014 | 0.025 | —    | —    |

Table 2

|                               | Yield point in kg./mm. <sup>2</sup> | Tensile strength in kg./mm. <sup>2</sup> | Elongation in Percent | Reduction of area in Percent | Hardness in Brinell | V-notch Charpy value in kg.-m./cm. <sup>2</sup> |      |         |      | Rotary bending fatigue limit in kg./mm. <sup>2</sup> |            |                             |                  | Corrosion in mm./half year |  |
|-------------------------------|-------------------------------------|------------------------------------------|-----------------------|------------------------------|---------------------|-------------------------------------------------|------|---------|------|------------------------------------------------------|------------|-----------------------------|------------------|----------------------------|--|
|                               |                                     |                                          |                       |                              |                     | Room temperature                                |      | —20° C. |      | Smooth                                               | With notch | Smooth, corroded with water | Exposed outdoors | Sprayed with salt water    |  |
|                               |                                     |                                          |                       |                              |                     | L                                               | C    | L       | C    |                                                      |            |                             |                  |                            |  |
|                               |                                     |                                          |                       |                              |                     |                                                 |      |         |      |                                                      |            |                             |                  |                            |  |
| Rail of the present invention | 76.8                                | 130.6                                    | 11.6                  | 20.9                         | 374                 | 8.12                                            | 3.89 | 6.52    | 3.51 | 55.0                                                 | 28.0       | 31.0                        | 0.022            | 0.55                       |  |
| Current carbon steel rail     | 43.3                                | 87.5                                     | 13.8                  | 23.5                         | 240                 | 1.30                                            | 0.65 | —       | —    | 32.0                                                 | 15.0       | 20.0                        | 0.078            | 0.95                       |  |

Table 3

|                                                       | Air-cooled to the room temperature after being directly fed and rolled | Air-cooled to the room temperature after being reheated and rolled | Slow cooling from each temperature during air cooling after finish-rolling |         |         |         |         |         |
|-------------------------------------------------------|------------------------------------------------------------------------|--------------------------------------------------------------------|----------------------------------------------------------------------------|---------|---------|---------|---------|---------|
|                                                       |                                                                        |                                                                    | 500° C.                                                                    | 550° C. | 600° C. | 650° C. | 700° C. | 750° C. |
| Tensile strength in kg./mm. <sup>2</sup> .....        | 122.4                                                                  | 135.0                                                              | 133.1                                                                      | 133.3   | 132.9   | 134.0   | 133.8   | 134.1   |
| Elongation in percent.....                            | 2.3                                                                    | 5.8                                                                | 6.7                                                                        | 7.6     | 9.9     | 13.0    | 11.8    | 11.9    |
| Reduction of area in percent.....                     | 4.7                                                                    | 8.7                                                                | 12.8                                                                       | 14.5    | 19.9    | 25.2    | 28.7    | 28.3    |
| V-notch Charpy value in kg.-m./cm. <sup>2</sup> ..... | 7.2                                                                    | 7.7                                                                | 7.8                                                                        | 7.7     | 7.8     | 8.1     | 8.1     | 8.2     |
| Hardness in Brinell.....                              | 385                                                                    | 382                                                                | 376                                                                        | 375     | 373     | 372     | 363     | 367     |

As apparent from these results, as compared with the current carbon steel rail, the corrosion-resistant high tensile strength rail of the present invention has a yield point, tensile strength and fatigue limit 1.5 to 1.8 times as high, an elongation and reduction of area not substantially different, an impact value several times as high and a much higher low-temperature impact value. On the other hand, the corrosion-resistance of the rail of the present invention is more than three times as high. In the process for producing rails according to the present invention, reheating after blooming and slow cooling treatments after the finish-rolling are the most essential conditions. These operations improve the elongation and reduction of area values. Current carbon steel rails are not affected by reheating and slow cooling. That is, current rails have substantially the same mechanical properties when slowly cooled to room temperature after being rolled as they do when they are not slowly cooled. Therefore, with reference to Tables 2 and 3, as compared with current carbon steel rails under the same conditions, i.e. slowly cooled to room temperature after being rolled, the rail of the present invention has a much higher tensile strength and hardness but is lower in elongation and reduction of area. It is therefore evident, that according to the present invention, a very high tensile strength is obtained, hardness and strength are not altered or are higher, the rates of elongation and reduction of area are equal to those of current carbon steel rails, and high corrosion-resistance is attained. Further, it is seen in Table 3 that the elongation and reduction of area of the rail of the present invention are more improved by reheating before rolling than by directly rolling and are further improved by slow cooling from 500 to 750° C. after finish-rolling.

What we claim is:

1. A method of manufacturing steel rail which is high in tensile strength and anti-corrosiveness which comprises subjecting a steel containing from 0.05 to 0.25% carbon, from 2.0 to 6.0% chromium, less than 1.5% manganese, from 0.1 to 1.0% molybdenum and less than 1.0% silicon as main components, adding an element selected from a group consisting of less than 1.0% nickel, less than 0.5% vanadium, less than 0.5 niobium, less than 1.0% copper, less than 0.01% boron, less than 0.5% titanium, and mixture thereof and the rest being Fe, to a blooming rolling, subjecting the bloomed material to a finish-rolling, to rail, subjecting the rail to an air-cooling after the finish-rolling, putting the rail into a heat-keeping furnace, when the temperature of the rail becomes 500 to 750° C., in which the rail is gradually cooled from a range of 500 to 750° C. down to a range of 150 to 200° C. for more than 7 hours.

15 to a rolling temperature, at which temperature said steel is rolled in rail, and then gradually cooling said rail from a temperature above 500 to 700° C. down to 150° C., over a period in excess of 7 hours.

2. A method as in claim 1, in which a mixture of elements selected from a group consisting of less than 1.0% nickel, less than 0.5% vanadium, less than 1.0% copper, less than 0.01% boron, less than 0.5% titanium and less than 0.5% niobium are added to the main components of the steel.

3. A method of manufacturing steel rail which is high in tensile strength and anti-corrosiveness which comprises subjecting a steel containing from 0.05 to 0.25% carbon, from 2.0 to 6.0% chromium, less than 1.5% manganese, from 0.1 to 1.0% molybdenum and less than 1.0% silicon as main components, adding an element selected from a group consisting of less than 1.0% nickel, less than 0.5% vanadium, less than 0.5 niobium, less than 1.0% copper, less than 0.01% boron, less than 0.5% titanium, and mixture thereof and the rest being Fe, to a blooming rolling, subjecting the bloomed material to a finish-rolling, to rail, subjecting the rail to an air-cooling after the finish-rolling, putting the rail into a heat-keeping furnace, when the temperature of the rail becomes 500 to 750° C., in which the rail is gradually cooled from a range of 500 to 750° C. down to a range of 150 to 200° C. for more than 7 hours.

References Cited by the Examiner

UNITED STATES PATENTS

|           |        |                 |       |        |
|-----------|--------|-----------------|-------|--------|
| 1,277,372 | 9/1918 | Brunner         | ----- | 148—12 |
| 1,721,555 | 7/1929 | Hamilton et al. | ----- | 75—126 |
| 1,925,029 | 8/1933 | Brunner         | ----- | 148—12 |

FOREIGN PATENTS

|         |        |                |
|---------|--------|----------------|
| 797,762 | 2/1936 | France.        |
| 324,686 | 1/1930 | Great Britain. |
| 340,819 | 1/1930 | Great Britain. |
| 517,118 | 1/1940 | Great Britain. |
| 731,684 | 6/1955 | Great Britain. |

55 DAVID L. RECK, Primary Examiner.

P. WEINSTEIN, Assistant Examiner.